

## UNITED STATES PATENT OFFICE

2,075,283

## PRODUCTION OF MAGNETIZABLE ALLOY

Albert Heinzel, Oppau, and Franz Duftschmid, Heidelberg, Germany, assignors to I. G. Farben-industrie Aktiengesellschaft, Frankfort-on-the-Main, Germany

No Drawing. Application August 31, 1935, Serial No. 38,788. In Germany September 4, 1934

9 Claims. (Cl. 148—11.5)

The present invention relates to the production of magnetizable alloys.

We have found that alloys of nickel and iron acquire excellent magnetic properties, in particular a high initial and maximum permeability, by subjecting them during their working up into sheets, bands or wires to a cold working of more than 60 per cent, subjecting them to a softening annealing, then subjecting them to a slight cold working, advantageously of less than 20 per cent, to bring them to their final thickness and then subjecting them to a final annealing, preferably at temperatures above 700° C. The process according to this invention is especially suitable 15 for the preparation of highly magnetic alloys of iron and nickel alone, in particular for those containing from 40 to 50 per cent of nickel and from 60 to 50 per cent of iron, but may also be employed for nickel-iron alloys having one or more 20 other components in minor quantities, as for example cobalt, aluminium, silicon, titanium, chromium, molybdenum, tungsten, copper or manganese.

Especially favourable results are obtained when 25 the first cold working is very strong, as for example amounting to from 80 to 90 per cent, and the cold working before the final annealing is not much stronger than the cold working above which a recrystallization is caused by annealing. 30 For example a cold working of 5 per cent after a cold working of 80 per cent effects an increase of the initial permeability to three times the value, and a working of 10 per cent after a working of 80 per cent doubles the initial permeability which is obtained without employing the slight additional cold working.

A special improvement in the magnetic quality is obtained when the alloys, in contrast to the manner of working hitherto adopted, are not subjected to an intermediate annealing after the 40 hot working, as for example after the hot rolling, i. e. before the first cold working according to this invention.

Nickel-iron alloys which have been rolled with 45 severe cold working frequently have initial permeabilities of less than 1000, a very flat course of the permeability curve measured in low-magnetic fields and increased coercive force. Such alloys having unsatisfactory properties may be 50 greatly improved by slight cold working according to this invention. For example a band which has been cold rolled without intermediate annealing, has, after having been wound onto a core and after the core has been annealed, an initial permeability of only 1000. Even the very 55

slight cold working effected by simply unwinding the band from the core and rewinding it causes, after a repeated annealing, an increase in the initial permeability to 6000, a very steeply ascending permeability curve and a coercive force down to 0.02 Oersted. More severe cold working, as for example slight stretching or reduction in cross-section, as for example by rolling down by less than about 20 per cent, also effects an improvement of the magnetic properties by a multiple (see the statements in Example 2 below).

According to this invention especially favourable magnetic qualities are obtained by selecting a comparatively high temperature, preferably from 1100° to 1200° C. for the final annealing. 15 It is preferable to employ in the final annealing a temperature which is higher the lower the temperature employed in the previous annealing. For example if the previous annealing is carried out at 800° C., the initial permeability is 2000, the permeability for 0.02 Oersted is 10500 and the coercive force is 0.06 Oersted when the final annealing is carried out at 900° C. and the corresponding values are 6000, 41000 and 0.031 when the final annealing is carried out at 1200° C.

It has been found of special advantage to employ the process according to this invention for alloys which have been prepared by pressure and/or heat treatment without melting from metal powders obtained from the corresponding 30 metal carbonyls by thermal decomposition.

The favourable magnetic properties obtained according to this invention render nickel-iron alloys containing from 40 to 50 per cent of nickel especially suitable for example for the construction of precision measuring transformers because these alloys combine in themselves a high permeability with weak fields, a very low coercive power with high saturation and a high 35 electrical resistance.

The following examples will further illustrate the nature of this invention but the invention is not restricted to these examples.

## Example 1

An alloy containing 50 per cent of nickel and 50 per cent of iron is prepared from the metals obtained from their carbonyl compounds, by sintering the powdery mixture. The sinter block is consolidated under a forging hammer and then 50 worked up into a strip by hot and cold rolling; the cold working after the last intermediate annealing in this treatment results in a reduction in cross section of 80 per cent. The strip is then subjected to a softening annealing for 55

four hours at 1100° C. in an atmosphere of hydrogen (Sample I). A part of the annealed strip is further cold worked to the extent of 10 per cent (Sample II), and another part of the strip is cold worked to the extent of 5 per cent (Sample III) reduction in cross section. All three strips are then wound in the same way onto cores while strewing with magnesia powder and annealed for four hours in hydrogen at 1100° C. 10 The three strips have the following magnetic values:—

|                               | I     | II    | III   |
|-------------------------------|-------|-------|-------|
| Initial permeability          | 1800  | 3500  | 5500  |
| Permeability for 0.02 Oersted | 2750  | 6500  | 18500 |
| Maximum permeability          | 48200 | 66500 | 84000 |
| Coercive force in Oersted     | 0.08  | 0.058 | 0.038 |

20 The initial permeability is always extrapolated from measuring values down to below 0.001 Oersted.

*Example 2*

An alloy containing 50 per cent of nickel and 25 50 per cent of iron is prepared by sintering the metal powders obtained from carbonyls, consolidated by forging and then worked up into a strip by hot rolling and subsequent cold rolling with a 30 per cent reduction in cross section without 30 intermediate annealing. The strip is wound into cores which are then treated in the following manner, the annealing always being carried out in an atmosphere of hydrogen:—

| 35 | Treatment                                                         | Initial permeability | Permeability for 0.02 Oersted | Maximum permeability | Coercive force |
|----|-------------------------------------------------------------------|----------------------|-------------------------------|----------------------|----------------|
| 40 | Core of strip annealed at 1100° C.                                | 1000                 | 1800                          | 116300               | 0.081          |
| 45 | Annealed at 1100° C., unwound, rewound, and annealed at 1100° C.  | 3000                 | 80000                         | 134800               | 0.024          |
| 50 | Annealed at 1100° C., slightly stretched and annealed at 1100° C. | 4000                 | 36000                         | 84100                | 0.038          |
|    | Annealed at 1100° C., rolled 5 per cent and annealed at 1100° C.  | 4300                 | 26000                         | 95300                | 0.033          |
|    | Annealed at 1100° C., rolled 17 per cent and annealed at 1100° C. | 5000                 | 20500                         | 107400               | 0.040          |
|    | Annealed at 1100° C., rolled 22 per cent and annealed at 1100° C. | 3000                 | 9000                          | 51600                | 0.056          |

What we claim is:

1. A process for the production of magnetizable alloys substantially consisting of nickel and iron 55 which comprises reducing the raw material to its definite thickness by subjecting it to a cold working of more than 60 per cent, then to a softening annealing, then to a slight cold working and then to a final annealing.

60 2. A process for the production of magnetizable alloys substantially consisting of nickel and iron which comprises reducing the raw material to its

definite thickness by subjecting it to a cold working of from about 80 to 90 per cent, then to a softening annealing, then to a slight cold working and then to a final annealing.

3. A process for the production of magnetizable 5 alloys substantially consisting of nickel and iron which comprises reducing the raw material to its definite thickness by subjecting it to a cold working of from about 80 to 90 per cent, then to a softening annealing, then to a cold working 10 of less than 20 per cent, and then to a final annealing.

4. A process for the production of magnetizable 15 alloys substantially consisting of nickel and iron which comprises reducing the raw material to its definite thickness by subjecting it to a cold working of from about 80 to 90 per cent, then to a softening annealing, then to a cold working not much stronger than that above which a recrystallization 20 is caused by annealing and then to a final annealing.

5. A process for the production of magnetizable 25 alloys substantially consisting of nickel and iron which comprises reducing the raw material to its definite thickness by subjecting it to a cold working of more than 60 per cent then to a softening annealing, then to a slight cold working and then to a final annealing above the recrystallization 30 temperature.

6. A process for the production of magnetizable 35 alloys substantially consisting of nickel and iron which comprises reducing the raw material to its definite thickness by subjecting it to a cold working of more than 60 per cent, then to a softening annealing, then to a slight cold working and then to a final annealing at a temperature between 30 and 40 about 1100° and about 1200° C.

7. A process for the production of magnetizable 40 alloys substantially consisting of nickel and iron which comprises reducing the raw material, prepared by heat treatment without melting from metal powders obtained from the corresponding metal carbonyls by thermal decomposition, to its definite thickness by subjecting it to a cold working of more than 60 per cent, then to a softening 45 annealing, then to a slight cold working and then to a final annealing.

8. A process for the production of magnetizable 50 alloys containing of from 40 to 50 per cent of nickel and of from 60 to 50 per cent of iron which comprises reducing the raw material to its definite thickness by subjecting it to a cold working of more than 60 per cent, then to a softening annealing, then to a slight cold working and then to a final annealing.

9. A process as defined in claim 2, wherein the 55 final annealing step is carried out at a temperature which is higher the lower the temperature employed in the preceding annealing step.

ALBERT HEINZEL.  
FRANZ DUFTSCHMID.